

E. A. CUSTER.  
ART OF CASTING STEEL.  
APPLICATION FILED JUNE 3, 1910.

1,042,092.

Patented Oct. 22, 1912.



Witnesses:  
George H. Custer  
J. Herbert

Inventor  
Edgar A. Custer  
By his Attorneys  
Redding, Green & Austin

# UNITED STATES PATENT OFFICE

EDGAR A. CUSTER, OF PHILADELPHIA, PENNSYLVANIA, ASSIGNOR TO THE CUSTER SANDLESS CASTING COMPANY, OF PHILADELPHIA, PENNSYLVANIA, A CORPORATION OF DELAWARE.

## ART OF CASTING STEEL.

1,042,092.

Specification of Letters Patent. Patented Oct. 22, 1912.

Application filed June 3, 1910. Serial No. 564,885.

To all whom it may concern:

Be it known that I, EDGAR A. CUSTER, a citizen of the United States, residing in the city of Philadelphia, in the State of Pennsylvania, have invented certain new and useful Improvements in the Art of Casting Steel, of which the following is a specification, reference being had to the accompanying drawing, forming a part hereof.

On account of the excessive shrinkage which takes place in cast steel, when cooling slowly in sand molds, from a molten condition, it has been necessary heretofore to provide for each mold one or more sink heads, that is, temporary receptacles, connected with the mold, to contain a body of molten metal sufficient to fill the "pipe" or hollow which otherwise develops in the casting during the slow cooling. The casting thus becomes solid, the pipe or hollow being formed in the sink head where it does no harm. This process of casting steel, however, involves much expense as compared with the value of the metal in the casting; a much larger volume of metal than is actually required for the casting must be prepared, thereby involving additional expense in melting, and the sink head must be cut off from the casting and broken up for remelting, thereby involving much labor.

The present invention has for its object to produce solid steel castings without the use of sink heads and therefore to reduce very largely the cost of making steel castings as compared with methods now in use.

In accordance with the invention the steel casting is cooled quickly, as by being cast in an iron mold of sufficient bulk to rob the casting swiftly of its heat, rather than slowly, as in the usual method, and the point of pouring of the molten metal into the mold itself is moved progressively, so as to keep pace with the point of setting of the molten metal in the mold as it progresses from the bottom to the top or from one end to the other.

The invention will be more fully explained hereinafter with reference to the accompanying drawing which represents, partly in outline and partly in section, so much of a mold and of the process of casting therein as is necessary to enable the invention to be understood.

The mold *a* is formed of such material,

preferably of iron, and is of such bulk that it will rob the casting swiftly of its heat, causing the molten metal to cool so rapidly that it will set as it is poured into the mold. The mold is provided with a runner *b* which extends practically throughout the full length of the casting and communicates with the chamber *c* of the mold practically throughout its length, through a long gate or a long succession of gates *d*. The metal is poured into the mold somewhat slowly and sets as it is poured. If the pouring of the metal should be stopped at any point, when only a portion of the chamber of the mold had been filled, as indicated at *e*, the metal would shrink and set with a conical cavity or pipe *f* in its upper surface. The pouring of the metal, however, is not checked but is continuous, keeping pace with the rise of the line of setting of the metal in the chamber of the mold until the chamber of the mold is completely filled and the casting is fully formed, the cavity or pipe which would otherwise be formed at the top of the casting being filled from the top of the gate. The volume of molten metal which may remain at the top of the casting when the chamber is filled is small and the shrinkage is therefore so slight in comparison with that of the remainder of the casting that its effect is negligible and the final result is a solid casting from end to end.

From the above description it will be understood that wherever it is stated that the metal is poured so as to keep pace with the progressive setting of the metal in the mold that it is meant that the pouring of the metal is continued as the setting of the metal in the mold progresses and in proportion to the progress of the line of setting of the metal in the mold.

It will be understood that the pouring of the metal so as to keep pace with the progression of the line of setting can be accomplished by varying the size of the runner and gate or gates to suit the shape and size of the chamber within the mold. It will also be understood that one or more runners with the necessary gates may be provided as the nature of the casting may require.

It will be seen that the upper part of the runner or runners of the mold contains a sufficient quantity of molten metal to in-

sure the complete filling of the mold chamber and that the quantity of metal which must be melted and poured for each casting, in excess of that which actually enters into the casting, is very small as compared with the quantity which must be melted and poured when the casting is allowed to cool slowly in a sand mold and a large sink head is necessary to insure the filling of the pipe formed by the gradual and consequent slow setting of the body of the casting, as in the methods heretofore generally in use. It will also be seen that the labor necessary to handle the superfluous metal and prepare it for remelting is small as compared with that necessary to handle and prepare for remelting the large masses of metal contained in the usual sink heads.

I claim as my invention:

1. The improvement in the art of casting steel which consists in cooling the metal as it fills the matrix of the mold so that the

metal will set throughout the casting at the same rate at which it is poured.

2. The improvement in the art of casting steel which consists in cooling the metal as it fills the mold quickly and progressively and pouring the metal so as to keep pace with the progressive setting of the metal in the mold.

3. The improvement in the art of casting steel which consists in continuously pouring the metal into the mold chamber through a long gate and cooling the metal as it fills the mold quickly and progressively, the pouring of the metal into the mold being at the same rate at which the metal sets.

This specification signed and witnessed this 26th day of May, A. D. 1910.

EDGAR A. CUSTER.

Signed in the presence of—

AMBROSE L. O'SHEA,  
ELLA J. KRUGER.